

Feb. 27, 1923.

1,446,879

J. J. COFFEY

RIVET SET AND METHOD OF MAKING SAME

Filed June 15, 1921

FIG. 1.



FIG. 2.



Inventor  
John James Coffey,

By Watson, Tait, Morse & Grindle,

Attn: [unclear]

## UNITED STATES PATENT OFFICE.

JOHN JAMES COFFEY, OF BETHLEHEM, PENNSYLVANIA, ASSIGNOR TO BETHLEHEM STEEL COMPANY, OF BETHLEHEM, PENNSYLVANIA, A CORPORATION OF PENNSYLVANIA.

## RIVET SET AND METHOD OF MAKING SAME.

Application filed June 15, 1921. Serial No. 477,743.

To all whom it may concern:

Be it known that I, JOHN JAMES COFFEY, a citizen of the United States, and resident of Bethlehem, county of Northampton and State of Pennsylvania, have invented certain new and useful Improvements in Rivet Sets and Methods of Making Same, of which the following is a specification.

This invention relates to a rivet set for use in pneumatically operated riveting machines and is designed to improve the structural characteristics of the material in an old and well known form of rivet set, such as steel, giving it greater strength, efficiency and lasting qualities. One essential feature of it is that the longitudinally extending central core is hard while the surrounding integral exterior portion is tough and fatigue resisting from the contact end to a point beyond that where breakage in use usually occurs in such devices. The invention consists in the structurally novel product or article and the method of producing it. The novel features will be understood from the following description and claims taken with the drawing.

In the drawing:

Figure 1 is a longitudinal section of a rivet set having an old and well known outward form, but showing small holes or connecting passageways drilled therein, and

Figure 2 is a cross section on the line 2—2 of Figure 1.

As is well known in the art, the blow of the piston of the pneumatic riveter is limited to a comparatively small central circular portion of the end surface 10 of the shank or reduced cylindrical portion 11, and the tendency to break under the strains of use is greatest at the inner end of the shank or reduced cylindrical portion 11 at the point where it integrally joins the enlarged flange 12 of the body portion. It is necessary for efficient use that the contact surface shall be hard, and to this end the common practice has been to subject the article to a treatment which hardens it throughout, but this has proved unsatisfactory because it makes the metal brittle and the upper shank or reduced cylindrical portion 11 often breaks, thus not only destroying its usefulness but scoring and injuring the cylinder of the pneumatic riveter. The present in-

vention secures all of the hardness desired in the central contact portion while providing that hard core throughout the shank which is likely to break with integral surrounding and supporting metal which is sufficiently tough and strong to sustain the strains in use and prevent breakage. To this end a hole or passageway 13 is drilled centrally in the contact end 10 longitudinally of the rivet set through the shank or cylindrical portion 11 to the point 14 in the enlarged cylindrical part 15 of the body portion beyond the flange 12. Somewhat smaller radial holes or passageways 16, preferably four in number, are then drilled in the cylindrical portion 15 equally spaced around the circumference and at their inner ends entering the longitudinal passageway 13 at its inner end. The article or tool is then heated to a temperature of approximately 1460 degrees F. and water is forced under pressure into the radial holes or passageways 16 and of course travels along passageway 13 and is discharged at the contact end 10. This rapid passage of water through the interior of the tool from the inner end of hole 13 to its outer end of course causes a rapid and uniform cooling from the center line outward, and when the temperature of the outer walls of the tool has fallen to about 900 degrees F., further cooling by water is discontinued, and the tool is then plunged in oil and is allowed to cool further in a normal way. The result of this treatment or operation is to leave the central longitudinal core portion hard or of a martensitic structure surrounded by a sheath of material thickness composed of metal which is tough and fatigue resisting or of sorbitic structure extending out to the surface.

Having thus described my invention, what is claimed as new and desired to be secured by Letters Patent is:

1. A rivet set having a hard core of martensitic structure longitudinally of the shank extending to the end contact surface and an integral surrounding sheath or body of metal which is tough and fatigue resisting in character and of sorbitic structure.
2. A rivet set having a small central longitudinal hole or passageway in the shank from the contact end surrounded by a hard metal core of martensitic structure and an

outer integral sheath of metal around the core which is tough and fatigue resisting in character and sorbitic in structure.

3. As an article of manufacture, a rivet set for pneumatic riveters having radial holes or passageways in its body portion entering the inner end of a central longitudinal passageway extending out through the shank to its contact end, a hard core of 10 martinsitic structure surrounding said longitudinal passageway and an integral sheath or body of metal which is tough and fatigue resisting in character and sorbitic in structure surrounding said hard core.

15. 4. The method of treating a rivet set to give it desired characteristics which consists in heating it to a high temperature, rapidly cooling its shank portion from its center line outward to such an extent as to form 20 a hard central core and then so cooling the entire body that the sheath of metal surrounding the hard central core will be tough and fatigue resisting.

25. 5. The method of treating a rivet set for pneumatic riveters which consists in heating it to a temperature of approximately 1460 degrees F., rapidly cooling its shank portion from its center line outward until the temperature of the outer surface falls to

about 900 degrees F., then dipping it in oil 30 and allowing it to cool to normal temperature.

6. The method of treating a metal rivet set to give it desired characteristics which 35 consists in heating it to a high temperature and then passing a stream of water under pressure through a small central passageway extending from within the body portion to the contact end of the shank until the central core portion of the metal extending only 40 part way to the surface has become hard and of martinsitic structure and then ceasing the water cooling and plunging the article in oil and allowing it to cool.

7. The method of treating a metal rivet 45 set to give it desired characteristics which consists in heating it to a temperature of approximately 1460 degrees F., forcing water under pressure through laterally extending passageways in the body portion and a 50 connected central passageway out through the contact end of the shank until the temperature of the outer surface falls to about 900 degrees F., and then plunging it in oil.

In testimony whereof I hereunto affix my 55 signature.

JOHN JAMES COFFEY.